

# United States Patent

[19]

Kosmos

[11] 3,850,766

[45] Nov. 26, 1974

[54] ELECTROPLATING BRIGHTENER  
COMPOSITIONS AND PROCESS

[75] Inventor: John C. Kosmos, Hasbrouck  
Heights, N.J.

[73] Assignee: Sterwin Chemicals, Inc., New York,  
N.Y.

[22] Filed: Mar. 28, 1974

[21] Appl. No.: 455,526

[52] U.S. Cl. 204/50 Y, 204/DIG. 2, 204/55 Y

[51] Int. Cl. C23b 5/10, C23b 5/46

[58] Field of Search 204/50 Y, 50 R, 55 Y, 55 R,  
204/DIG. 2

[56] References Cited

UNITED STATES PATENTS

2,196,588 4/1940 Hull ..... 204/55 Y

|           |         |                 |          |
|-----------|---------|-----------------|----------|
| 2,233,500 | 3/1941  | Westbrook ..... | 204/55 Y |
| 3,088,884 | 5/1963  | Passal .....    | 204/55 Y |
| 3,285,840 | 11/1966 | Lindemann ..... | 204/55 R |

Primary Examiner—G. L. Kaplan  
Attorney, Agent, or Firm—Elmer J. Lawson; William  
G. Webb

[57]

## ABSTRACT

Zinc or cadmium electroplating brightener compositions for addition to alkaline cyanide electroplating baths comprising an aqueous solution of corn syrup or glucose, vanillin, veratraldehyde, sodium lignin sulfonate and sodium bisulfite.

12 Claims, No Drawings

## ELECTROPLATING BRIGHTENER COMPOSITIONS AND PROCESS

This invention relates to compositions and processes useful in the art of electroplating. More specifically, it relates to compositions useful as brightener additives to alkaline cyanide zinc or cadmium electroplating baths and to processes of bright electroplating using said compositions.

It is known in the art to use as brighteners in electroplating baths such materials as waste sulfite liquors (U.S. Pat. No. 1,544,726); various sulfonic acid derivatives (including the alkali metal salts thereof) such as alkyl-substituted-aromatic sulfonic acids (U.S. Pat. No. 2,312,097), sulfonic acid derivatives of phenols (U.S. Pat. No. 1,607,870); lignin sulfonic acid and metal salts thereof including the sodium salt (U.S. Pat. Nos. 2,740,754; 2,872,392 and 3,146,178); certain aromatic aldehydes such as anisic aldehyde (U.S. Pat. No. 2,740,754); and various proteins, such as peptone (U.S. Pat. No. 2,799,635) or hydrolyzed meat protein (U.S. Pat. No. 3,751,348).

It has now been surprisingly found that a combination in an aqueous medium of corn syrup or glucose, vanillin, veratraldehyde and sodium lignin sulfonate (together with a molar equivalent amount of sodium bisulfite equal to the molar equivalent amount of vanillin and veratraldehyde which is used to solubilize the vanillin and veratraldehyde through the bisulfite addition compound), when used as an additive to alkaline cyanide zinc or cadmium plating baths, provides advantages over the use of the separate brightener ingredients when used alone.

Thus, although sodium lignin sulfonate does provide a brightening effect, the degree of brilliance obtained over a range of low to high current densities is not uniform when the material is used alone. On the other hand, when combined with the other ingredients of the present invention, consistently brilliant deposits are obtained at both high and low current densities, and furthermore the inclusion of the sodium lignin sulfonate with the other ingredients tends to extend the lifetime of the bath over its normal limit. Glucose or corn syrup, when used alone, provide only a small degree of brightening, and like sodium lignin sulfonate, give inconsistent results over broad ranges of current densities. Vanillin used alone also provides a brightening effect, but consistent results are only obtained at high current densities, and darkening of the deposit is caused at low current densities. Veratraldehyde alone causes pitting of the deposit at low current densities, and furthermore the tolerance of the bath to impurities is diminished relative to results obtained with the instant compositions. As indicated hereinbelow ammonium heptamolybdate, a known electroplating brightener, can also be used in conjunction with the compositions of the present invention. However, this material used alone causes blistering of the deposit at high current densities and fails to deposit at low densities and thus is useful alone only at intermediate current densities. On the other hand, the novel combination of ingredients used in the practice of the present invention provides consistently good results, in terms of brightening effect, tolerance to impurities, extended bath life and adherence, over a broad range of current densities.

Moreover, the bath additive compositions useful in the practice of the present invention can, if desired, be

used in conjunction with other agents known to provide added brilliance to the electrodeposit such as molybdate salts, for example ammonium heptamolybdate, or with polysulfides in the case of cyanide zinc baths, for example ammonium, sodium or potassium polysulfide, which are used to combine with metallic impurities in the electroplating bath and thereby serve to prevent impurities from interfering with deposition of the pure metal.

10 The bath additive compositions provided by the present invention are preferably prepared in concentrated form, and in use are further diluted with water for addition to new or old working electroplating solutions in amounts to be described hereinafter. The concentrated form contains from 1.0 to 4.3 pounds/gallon of sodium lignin sulfonate, about 0.9 pound/gallon of veratraldehyde, from 0.1 to 2.2 pounds/gallon of vanillin, from 1.5 to 4.5 pounds/gallon of corn syrup or glucose, and a molar equivalent amount of sodium bisulfite corresponding to the total weight of the vanillin and veratraldehyde. Since, as will be described hereinafter, the additive compositions can be made up in varying concentrations ranging from dilute solutions that can be added directly to the plating bath to more concentrated solutions that require further dilution before addition to the plating bath, the compositions can also be described in terms of the relative amounts of the separate ingredients. Thus, relative to the veratraldehyde present, the operative amounts of the separate ingredients, expressed in parts by weight, are:

|                         |         |
|-------------------------|---------|
| Sodium lignin sulfonate | 1.1-4.8 |
| Veratraldehyde          | 1.0     |
| Vanillin                | 0.1-2.5 |
| Corn syrup or glucose   | 1.7-5.0 |

and a molar equivalent amount of sodium bisulfite corresponding to the total molar equivalent amount of the vanillin and veratraldehyde.

40 The compositions can be used in either barrel or still plating procedures, and when employed in barrel or still plating of cadmium, they may optionally contain, in addition to the ingredients described above, from 0.018 to 0.4 pound/gallon of ammonium heptamolybdate (or from 0.02 to 0.4 part by weight relative to veratraldehyde) to improve the brilliance of the deposit. When employed in barrel or still plating of zinc, they may optionally contain, respectively, from 0.018 to 0.4 pound/gallon (0.02 to 0.4 part by weight relative to veratraldehyde) or from 0.015 to 0.18 pound/gallon (0.017 to 0.2 part by weight relative to veratraldehyde) of ammonium heptamolybdate.

45 A preferred composition contains from 1.35 to 3.2 pounds/gallon of sodium lignin sulfonate, 0.9 pound/gallon of veratraldehyde, from 0.18 to 1.35 pounds/gallon of vanillin, from 2.0 to 4.0 pounds/gallon of corn syrup or glucose, and a molar equivalent amount of sodium bisulfite equal to the total amount of vanillin and veratraldehyde. When ammonium heptamolybdate is used to enhance the brilliance of the deposit in cadmium barrel or still plating, it is preferred to use from 0.045 to 0.27 pound/gallon of the heptamolybdate, and when the heptamolybdate is used in barrel or still plating of zinc, it is preferred to use, respectively, from 0.045 to 0.27 pound/gallon or from 0.018 to 0.18 pound/gallon of the heptamolybdate. Expressed in parts by weight relative to veratraldehyde, the preferred composition contains:

|                         |         |
|-------------------------|---------|
| Sodium lignin sulfonate | 1.5-3.5 |
| Veratraldehyde          | 1.0     |
| Vanillin                | 0.2-1.5 |
| Corn syrup or glucose   | 2.2-4.5 |

5

|                    |               |
|--------------------|---------------|
| Zinc cyanide       | 8.0 oz./gal.  |
| Sodium cyanide     | 5.6 oz./gal.  |
| Sodium hydroxide   | 8-10 oz./gal. |
| Sodium polysulfide | 0.12 oz./gal. |

and a molar equivalent amount of sodium bisulfite equal to the total amount of vanillin and veratraldehyde. When ammonium heptamolybdate is used in barrel or still plating of cadmium or in barrel plating of zinc, a preferred amount is from 0.05 to 0.3 part by weight relative to the veratraldehyde, and when it is used in still plating of zinc, a preferred amount is from 0.02 to 0.2 part by weight relative to veratraldehyde.

In use, the concentrates described above are diluted with three parts of water and added to the electroplating bath. In the case of new baths, an amount of the so-diluted solution to provide 1-2 percent by volume of the final plating solution is used, whereas in the case of old working baths, it is sufficient to add one-half percent by volume of the diluted concentrate.

The compositions of the invention, when used in barrel plating of cadmium, give best results at 9-12 volts E.M.F., while in barrel plating of zinc, best results are obtained at 10-15 volts E.M.F. In still plating of cadmium, a current density of 5-80 amperes/ft<sup>2</sup> can be used with advantage, a current density of 10-40 amperes/ft<sup>2</sup> being preferred. In still plating of zinc, good results are obtained at current densities of 10-80 amperes/ft<sup>2</sup>, a preferred range being 20-50 amperes/ft<sup>2</sup>. In all cases, plating is advantageously carried out at temperatures from 70°-90°F.

Having described the general manner of making and using the invention, the best mode of carrying out the invention is described by the following specific examples.

#### EXAMPLE 1

##### Basic Concentrate

A concentrate containing the following ingredients:

|                         |      |             |
|-------------------------|------|-------------|
| Sodium lignin sulfonate | 1.49 | pounds/gal. |
| Veratraldehyde          | 0.9  | pound/gal.  |
| Vanillin                | 0.6  | pound/gal.  |
| Corn syrup              | 2.08 | pounds/gal. |
| Sodium bisulfite        | 0.84 | pound/gal.  |

is prepared as follows:

A container of adequate size is charged with about 40 percent of the necessary quantity of water at 140°-150°F., and the sodium lignin sulfonate is added with stirring, followed by the corn syrup which is previously warmed to about 120°F. The vanillin and veratraldehyde are liquified by warming together on a hot water bath, and the liquid melt is added to the main mixture with stirring. The sodium bisulfite is then added slowly with stirring, and stirring is continued until all material is dissolved. Sufficient water is added to give the desired final volume, the solution is cooled to below 100°F., and then packed with stirring in polyethylene containers.

##### A. Zinc Barrel or Still Plating Composition

The concentrate so-prepared is diluted with three parts of water, and 10 to 20 gallons of the diluted solution are added to 1,000 gallons of a standard zinc cyanide bath containing:

The so-prepared bath when used in barrel plating at 10-15 volts E.M.F. at 70°-90°F. for 20-25 minutes gives an even, bright deposit of about 0.0002 inch thickness.

The same bath when used in still plating at a current density of 20-50 amperes/ft<sup>2</sup> at 70°-90°F. for 6-10 minutes gives an even, bright deposit of 0.0002 inch thickness.

##### B. Cadmium Barrel Plating Composition

The concentrate described in Example 1 above is diluted with three parts of water, and 10-20 gallons of the diluted solution are added to 1,000 gallons of a cadmium barrel plating solution containing:

|                  |                    |
|------------------|--------------------|
| Cadmium oxide    | 3.0 oz./gal.       |
| Sodium cyanide   | 10.4-13.4 oz./gal. |
| Sodium hydroxide | 1.0 oz./gal.       |

25 The bath so-prepared, when used in the barrel plating of cadmium at 9-12 volts E.M.F. at 70°-90°F. for 10-15 minutes gives an even, bright deposit of about 0.0002 inch thickness.

##### C. Cadmium Still Plating Composition

30 The concentrate described in Example 1 above is diluted with three parts of water, and 10-20 gallons of the diluted solution are added to 1,000 gallons of a cadmium still plating solution containing:

|                |                    |
|----------------|--------------------|
| Cadmium oxide  | 3.0 oz./gal.       |
| Sodium cyanide | 10.4-18.4 oz./gal. |

35 The bath so-prepared, when used in the still plating of cadmium at 10-40 amperes/ft<sup>2</sup> at 70°-90°F. for 5 minutes gives an even, bright deposit of about 0.002 inch thickness.

#### EXAMPLE 2

40 45 To the basic concentrate described in Example 1 above is added 0.06 pound/gallon (about 4 grams/liter) of ammonium heptamolybdate. The concentrate so-obtained is diluted with three parts of water, and 10-20 gallons of the diluted solution are added, respectively, to 1,000 gallons of the solutions described in Examples 1B and 1C above. The baths so-obtained in each case when used, respectively, in barrel plating and still plating of cadmium under the conditions described in Examples 1B and 1C, respectively, give deposits similar to those described in Examples 1B and 1C, respectively, but having improved brilliance thereover.

#### EXAMPLE 3

50 55 To the basic concentrate described in Example 1 above is added 0.03 pound/gallon (about 2 grams/liter) of ammonium heptamolybdate. The concentrate so-obtained is diluted with three parts of water, and 10-20 gallons of the diluted solution are added to 1,000 gallons of the solution described in Example 1A above. The bath so-obtained when used in still plating of zinc under the conditions described in Example 1A gives a deposit similar to that described in Example 1A but having improved brilliance thereover.

## EXAMPLE 4

To the basic concentrate described in Example 1 is added 0.06 pound/gallon (about 4 grams/liter) of ammonium heptamolybdate. The concentrate so-obtained is diluted with three parts of water, and 10-20 gallons of the diluted solution are added to 1,000 gallons of the solution described in Example 1A above. The bath so-obtained when used in barrel plating of zinc under the conditions described in Example 1A gives a deposit similar to that obtained in Example 1A but having improved brilliance thereover.

I claim:

1. In a process for bright plating of zinc or cadmium from aqueous alkaline cyanide electroplating baths, the improvement which comprises adding to said baths an aqueous composition containing, in parts by weight:

|                         |         |
|-------------------------|---------|
| Sodium lignin sulfonate | 1.1-4.8 |
| Veratraldehyde          | 1.0     |
| Vanillin                | 0.1-2.5 |
| Corn syrup or glucose   | 1.7-5.0 |

and a molar equivalent amount of sodium bisulfite equal to the total molar equivalent amount of the vanillin and veratraldehyde.

2. In a process for barrel or still bright plating of cadmium or barrel plating of zinc from aqueous alkaline cyanide electroplating baths, the improvement which comprises adding to said baths an aqueous composition containing, in parts by weight:

|                         |          |
|-------------------------|----------|
| Sodium lignin sulfonate | 1.1-4.8  |
| Veratraldehyde          | 1.0      |
| Vanillin                | 0.1-2.5  |
| Corn syrup or glucose   | 1.7-5.0  |
| Ammonium heptamolybdate | 0.02-0.4 |

and a molar equivalent amount of sodium bisulfite equal to the total molar equivalent amount of the vanillin and veratraldehyde.

3. In a process for still bright plating of zinc from aqueous alkaline cyanide electroplating baths, the improvement which comprises adding to said baths an aqueous composition containing, in parts by weight:

|                         |           |
|-------------------------|-----------|
| Sodium lignin sulfonate | 1.1-4.8   |
| Veratraldehyde          | 1.0       |
| Vanillin                | 0.1-2.5   |
| Corn syrup or glucose   | 1.7-5.0   |
| Ammonium heptamolybdate | 0.017-0.2 |

and a molar equivalent amount of sodium bisulfite equal to the total molar equivalent amount of the vanillin and veratraldehyde.

4. A process according to claim 1 wherein the bath additive composition contains, in parts by weight:

|                         |         |
|-------------------------|---------|
| Sodium lignin sulfonate | 1.5-3.5 |
| Veratraldehyde          | 1.0     |
| Vanillin                | 0.2-1.5 |
| Corn syrup or glucose   | 2.2-4.5 |

and a molar equivalent amount of sodium bisulfite equal to the total molar equivalent amount of the vanillin and veratraldehyde.

5. A process according to claim 2 wherein the bath additive composition contains, in parts by weight:

|                         |          |
|-------------------------|----------|
| Sodium lignin sulfonate | 1.5-3.5  |
| Veratraldehyde          | 1.0      |
| Vanillin                | 0.2-1.5  |
| Corn syrup or glucose   | 2.2-4.5  |
| Ammonium heptamolybdate | 0.05-0.3 |

and a molar equivalent amount of sodium bisulfite equal to the total molar equivalent amount of the vanillin and veratraldehyde.

6. A process according to claim 3 wherein the bath additive composition contains, in parts by weight:

|                         |          |
|-------------------------|----------|
| Sodium lignin sulfonate | 1.5-3.5  |
| Veratraldehyde          | 1.0      |
| Vanillin                | 0.2-1.5  |
| Corn syrup or glucose   | 2.2-4.0  |
| Ammonium heptamolybdate | 0.02-0.2 |

and a molar equivalent amount of sodium bisulfite equal to the total molar equivalent amount of the vanillin and veratraldehyde.

7. An electroplating brightener composition for addition to zinc or cadmium alkaline cyanide electroplating baths comprising an aqueous solution containing, in parts by weight:

|                         |         |
|-------------------------|---------|
| Sodium lignin sulfonate | 1.1-4.8 |
| Veratraldehyde          | 1.0     |
| Vanillin                | 0.1-2.5 |
| Corn syrup or glucose   | 1.7-5.0 |

and a molar equivalent amount of sodium bisulfite equal to the total molar equivalent amount of the vanillin and veratraldehyde.

8. An electroplating brightener composition for addition to cadmium barrel or still plating or zinc barrel plating alkaline cyanide electroplating baths comprising an aqueous solution containing, in parts by weight:

|                         |          |
|-------------------------|----------|
| Sodium lignin sulfonate | 1.1-4.8  |
| Veratraldehyde          | 1.0      |
| Vanillin                | 0.1-2.5  |
| Corn syrup or glucose   | 1.7-5.0  |
| Ammonium heptamolybdate | 0.02-0.4 |

and a molar equivalent amount of sodium bisulfite equal to the total molar equivalent amount of the vanillin and veratraldehyde.

9. An electroplating brightener composition for addition to zinc still plating alkaline cyanide electroplating baths comprising an aqueous solution containing, in parts by weight:

|                         |           |
|-------------------------|-----------|
| Sodium lignin sulfonate | 1.1-4.8   |
| Veratraldehyde          | 1.0       |
| Vanillin                | 0.1-2.5   |
| Corn syrup or glucose   | 1.7-5.0   |
| Ammonium heptamolybdate | 0.017-0.2 |

and a molar equivalent amount of sodium bisulfite equal to the total molar equivalent amount of the vanillin and veratraldehyde.

10. A composition according to claim 7 containing, in parts by weight:

|                         |         |
|-------------------------|---------|
| Sodium lignin sulfonate | 1.5-3.5 |
| Veratraldehyde          | 1.0     |

## -Continued

|                       |         |
|-----------------------|---------|
| Vanillin              | 0.2-1.5 |
| Corn syrup or glucose | 2.2-4.5 |

and a molar equivalent amount of sodium bisulfite equal to the total molar equivalent amount of the vanillin and veratraldehyde.

11. A composition according to claim 8 containing, in parts by weight:

|                         |          |
|-------------------------|----------|
| Sodium lignin sulfonate | 1.5-3.5  |
| Veratraldehyde          | 1.0      |
| Vanillin                | 0.2-1.5  |
| Corn syrup or glucose   | 2.2-4.5  |
| Ammonium heptamolybdate | 0.05-0.3 |

and a molar equivalent amount of sodium bisulfite

equal to the total molar equivalent amount of the vanillin and veratraldehyde.

12. A composition according to claim 9 containing, in parts by weight:

|    |                         |          |
|----|-------------------------|----------|
| 10 | Sodium lignin sulfonate | 1.5-3.5  |
|    | Veratraldehyde          | 1.0      |
|    | Vanillin                | 0.2-1.5  |
|    | Corn syrup or glucose   | 2.2-4.0  |
|    | Ammonium heptamolybdate | 0.02-0.2 |

and a molar equivalent amount of sodium bisulfite equal to the total molar equivalent amount of the vanillin and veratraldehyde.

\* \* \* \* \*

20

25

30

35

40

45

50

55

60

65